# EUROPEAN PATENT SPECIFICATION

(11) **EP 0 027 051 B1**
(45) Date of publication and mention of the grant of the patent: **11.07.1984**
(21) Application number: 80303526.0
(22) Date of filing: 07.10.1980
(51) Int. Cl.: C25B 11/10, C25B 1/34, C25D 17/10, C23C 15/00

(54) **Coated metal electrode with improved barrier layer and methods of manufacture and use thereof**
Beschichtete Metallelektrode mit Sperrschicht und Verfahren zu deren Herstellung und Verwendung
Electrode métallique plaquée à couche d'arrêt et procédés pour sa fabrication et son utilisation

(30) Priority: 08.10.1979 GB 7934856
(43) Date of publication of application: 15.04.1981
(73) Proprietor: ELTECH SYSTEMS CORPORATION, Boca Raton Florida 33434 (US)
(72) Inventor: Beer, Henri Bernard, B-2180 Heide Kalmthout (BE); Hinden, Jean Marcel, CH-1292 Chambesy (CH)
(74) Representative: Cronin, Brian Harold John

## Description

### Technical Field

The invention relates to electrodes for use in electrolytic processes, of the type having a substrate of a film-forming metal such as titanium, tantalum, zirconium, niobium, tungsten, aluminium and alloys containing one or more of these metals as well as silicon-iron alloys, coated with an electrocatalytic coating containing one or more platinum-group metals or their oxides possibly mixed with other oxides.

By "film-forming metal" is meant one which has the property that when connected as an anode in the electrolyte in which the coated anode is subsequently to operate, there rapidly forms a passivating oxide film which protects the underlying metal from corrosion by the electrolyte. These metals are also frequently referred to as "valve metals".

The invention is more particularly concerned with dimensionally-stable electrodes provided with an improved barrier or intermediate layer between the film-forming metal substrate and the electrocatalytic outer coating.

### Background Art

In early proposals (see for example U.K. Patent Specifications 855 107 and 869 865), a titanium electrode with a coating of platinum group metal was provided with an inert barrier layer of titanium oxide in the porous places of the coating, this barrier layer preferably being formed or reinforced by a heat treatment. Later, in U.K. Patent Specification 925 080, the inert barrier layer of titanium oxide was preformed by electrolytically treating or heating the titanium substrate in an oxidizing atmosphere prior to application of the platinum goup metal. The preforming of such a barrier layer was also advocated in U.K. Patent Specification 1 147 422 with a view to improving the anchorage of an active coating consisting of or containing platinum group metal oxides.

Later, the development of coatings formed of mixed crystals or solid solutions of co-deposited oxides of film-forming metals and platinum group metals (see U.S. Patent No. 3 632 498) provided commercially viable electrodes which revolutionized the chlor-alkali industry and have become widely used in other applications. With these electrodes, excellent performance was achieved without the need for a reinforced or preformed inert barrier or anchorage layer on the substrate and today it is generally accepted that the preformed or reinforced inert barrier layers are detrimental to performance. In retrospect, the early proposals for preformed or reinforced inert barrier layers appear to have been unsuccessful attempts to avoid defects which were inherent in the previous coatings rather than in the substrate.

Nevertheless, some proposals attempting to improve inert barrier layers have still been made, for example by applying a titanium oxide barrier layer from a solution containing Ti4+ ions. Again, this has been found to impair performance of the electrodes.

Another approach has been to provide a non-passivating barrier layer or intermediate layer underlying the active outer coating. Typical suggestions have been doped tin dioxide sub-layers; thin sub-layers of one or more platinum metals such as a platinum-iridium alloy; sub-layers of cobalt oxide or lead oxide, and so forth. Although various patents have claimed marginal improvements for these electrodes in specific applications, in practice none of these suggestions has led to any significant improvement or any widespread commercial use.

### Disclosure of the Invention

The invention concerns an electrode with a film-forming metal substrate having a porous outer electrocatalytic coating containing at least about 2 g/m² (as platinum group metal per projected surface area of the substrate) of at least one platinum group metal and/or oxide thereof possibly mixed with other metal oxides, and an improved non-passivating barrier layer between the substrate and coating.

According to the invention, this barrier layer is a preformed surface oxide film grown up from the film-forming base and having rhodium and/or iridium incorporated in the surface oxide film during formation thereof in an amount of up to 1 g/m² (as metal) per projected surface area of the substrate.

The surface oxide film of the barrier layer is rendered non-passivating by the incorporation of the rhodium and/or iridium as metal or as a compound, usually the oxide or a partially oxidized compound.

Another aspect of the invention is a method of manufacturing such an electrode in which the formation of the barrier layer involves the application of a very dilute acidic paint, i.e. one which contains a small quantity of a thermodecomposable iridium and/or rhodium compound that during decomposition and simultaneous formation of the surface film of film-forming metal oxide will be fully absorbed by this surface film, this dilute paint containing generally about 1-15 g/I of iridium and/or rhodium (as metal).

The paint used will typically include an organic solvent such as isopropyl alcohol, an acid (notably HCI, HBr or HI) or another agent (e.g. NaF) which attacks the film-forming metal and encourages the formation of film-forming metal oxide during the subsequent heat treatment, and one or more thermo-decomposable salts of iridium and/or rhodium. Usually this solution will be at least five times more dilute and preferably about 10 or more times dilute (in terms of its precious metal content) than the paint solution which may be used for the production of the outer porous electrocatalytic oxide coatings; this means that the quantity of iridium, and/or rhodium, will be reduced, e.g. to 1/5 or 1/10 or even 1/100th the amount of the corresponding platinum-group metal in the paint used for producing the outer coating for approximately the same quantity of solvent and acid.

The action of the acid or other agent which attacks or corrodes the film-forming metal and promotes the formation of the oxide film during the subsequent heat treatment is very important; without a suitable agent producing this effect, formation of the surface oxide film of the film-forming metal would be substantially hindered or inhibited.

It has been observed that by applying one coat of a given solvent/acid mixture to a film-forming metal base subjected previously to the usual cleaning and etching treatments and then heating after drying to drive off the solvent, a given quantity of film-forming metal oxide will be produced. This procedure can be repeated a number of times (usually four or five times for 4 ml HCL in 60 ml isopropyl alcohol applied to a titanium base, dried and heated to 500°C for ten minutes) before the growth of film-forming metal oxide during successive treatments becomes inhibited. The first layer of the integral surface oxide film formed will be relatively porous. This allows the subsequently-applied coat of the acid paint to penetrate this porous first layer during the drying phase so that the acid attacks the underlying film-forming metal. Ions of the film-forming metal are thus provided by the base for conversion to oxide during the subsequent heating, this oxide being partly formed within the pores of the first layer. The porosity of the resulting oxide film is thus reduced after each coating cycle until no more film-forming metal from the base can be converted to oxide. An extremely stable, relatively compact and impermeable film of film-forming metal oxide can thus be formed by the application of a limited number of coats of acid paint followed by drying and heating.

To prepare barrier layers according to the invention, each applied coat of paint includes such a small quantity of the iridium and'/or rhodium compound that the electrocatalyst formed by thermocomposition becomes fully incorporated in the integral surface film of film-forming metal oxide that is formed each time. Usually, each applied coat of the paint will contain at most about 0.2 g/m² or iridium and/or rhodium per projected surface area of the base, usually far less. Additionally, application of further layers of the dilute paint is stopped after the number of coats beyond which growth of the surface oxide film on the film-forming metal ceases or is inhibited. Thus, the optimum quantity of electrocatalytic agent in the dilute paint and the optimum number of coats to be applied to produce a satisfactory compact, impermeable barrier layer can be determined quite easily for any particular substrate, solvent/acid and electrocatalytic material. In many instances, two to ten layers of the very dilute paint will be applied, each followed by drying and heating from about 400 to 600°C for about 5 to 15 minutes, with the possible exception of the final layer which may be heated for a longer period - possibly several hours or days at 450-600°C in air or in a reducing atmosphere (e.g. ammonia/hydrogen).

When viewed by the naked eye or under a microscope, barrier layers produced in this manner on an etched or non-etched titanium base usually retain the same range of distinctive appearances as titanium oxide films prepared in the same manner which do not contain the iridium and/or rhodium electrocatalyst, typically a bright blue, yellow and/or red "interference" film colour.

The dilute acidic point solution used. to prepare the barrier layer according to the invention preferably only includes a thermo- decomposable iridium and/or rhodium compound, since the film-forming metal oxide component is provided by the base. However, the dilute paint may include small amounts of other components such as other platinum-group metals (ruthenium, palladium, platinum, osmium, in particular ruthenium), gold, silver, tin, chromium, cobalt, antimony, molybdenum, iron, nickel, manganese, tungsten, vanadium, titanium, tantalum, zirconium, niobium, bismuth, lanthanum, tellurium, phosphorous, boron, beryllium, sodium, lithium, calcium, strontium, lead and copper compounds and mixtures thereof. Usually, if any small quantity of a film-forming metal compound is used it will be a different metal to the film-forming metal substrate so as to contribute to doping of the surface film. Excellent results have been obtained with iridium/ruthenium compounds in a weight ratio of about 2:1, as metal. When such additives are included in the dilute paint composition, they will of course be in an amount compatible with the small amount of the main electrocatalyst, i.e. an iridium and/or rhodium compound, so that substantially all of the main electrocatalyst and additive is incorporated in the surface film of film-forming metal oxide. In any event, the total amount of iridium and/or rhodium and other metals is below 1 g/m², and usually below 0.5 g/m² and the extra metal will be present in a lesser amount than the rhodium and/or iridium. These iridium/rhodium compounds and other metal compounds may be thermodecomposable to form the metal or the oxide, but in neither case is it necessary to proceed to full decomposition. For example, barrier layers containing partially decomposed iridium chloride containing up to about 5% by weight of the original chlorine, have shown excellent properties. Barrier layers containing as little as 0.1 to 0.3 g/m² (as metal) of iridium and/or rhodium oxide/chloride in their surface films give excellent results. Tests have shown that a barrier layer containing 0.5 to 0.6 g/m² (as metal) or iridium produces an optimum affect in terms of the increased lifetime of the coated electrodes. Increasing the quantity of iridium above these values does not further increase the lifetime.

When a titanium substrate is used, the surface oxide film is found to be predominantly rutile titanium dioxide; presumably, the formation of rutile e.g. at about 400-500°C is catalysed by the rhodium and/or iridium in the dilute coating solution.

After formation of the improved barrier layer which is impermeable to electrolyte and to evolved oxygen, the porous outer electro- catalytic coating is applied using standard techniques, for example by applying over the preformed barrier layer a plurality of coats of a relatively concentrated solution containing a thermodecomposable platinum-group metal compound and heating. Each applied outer coat will contain at least 0.4 g/m² of the platinum-group metal per projected area of the substrate, and the coating procedure is repeated to build up an effective outer coating containing at least about 2 g/m² of the platinum-group metal(s), usually in oxide form. The coating components may be chosen to provide a coating consisting predominantly of a solid-solution of at least one film-forming metal oxide and at least one platinum-group metal oxide, as described in US Patent No. 3 632 498. Advantageously, the coating is a solid solution of ruthenium and titanium oxide having a ruthenium :titanium atomic ratio of from 1:1 to 1:4. In this instance, the coating consists of several superimposed layers typically having a micro-cracked appearance and is quite porous. Employing an improved barrier layer according to the invention with such a coating greatly improves the performance of the electrode in standard accelerated life-time tests in oxygen- evolution conditions. Predictably, in the conditions for normal commercial production of chlorine, the improved electrode will have a substantially longer lifetime since it is known that one of the reasons for failure of these electrodes after extended use in chlorine production is due to the action of oxygen on the substrate. Also, it will be possible to obtain the same lifetime with an appreciable reduction in the outer coating thickness, enabling a saving in the quantity of coating material used and in the labour and energy consumed for production.

The outer coating may also be formed of one or more platinum-group metals, for example a platinum-iridium alloy, useful for chlorate production and to a limited extent in diaphragm or membrane cells for chlorine production. With conventional Pt/ir coated electrodes, the coatings must be relatively thick (at least about 5 g/m²) to avoid passivation problems. With the improved barrier layer according to the invention, thinner and more porous layers of the platinum metals can be used without problems arising due to oxidation of the substrate, or the drawbacks associated with the previously known passive barrier layers of titanium oxide.

It is also possible to apply the outer coating by plasma-spraying a solid solution of a film-forming metal oxide and a platinum-group metal oxide. For example, a solid solution powder can be prepared by flame-spraying as described in US Patent No. 3 677 075 and this powder is then plasma-sprayed onto the base. Alternatively, the coating is applied by plasma-spraying at least one film-forming metal oxide over the preformed barrier layer and subsequently incorporating the platinum-group metal(s) and/or oxides thereof in the plasma-sprayed film-forming metal oxide, for example according to the procedure of US Patent No. 4 140 813. Again, the improved barrier layer increases lifetime and enables a reduction of the precious metal content of the coating.

In a preferred method of mass-producing the electrodes, a set of electrode sub-strates are subjected together to a series of pre-treatments including etching and formation of the barrier layer by dip-coating the set of substrates in said dilute solution and heating the set of sub- strates, and thereafter the outer electro- catalytic coating is applied to the substrates one at a time. This procedure obviates the drawback in commercial electrode coating plants associated with a "bottleneck" between the etching bath and the coating line. In the usual mass-production procedure, a set of substrates is pretreated by sandblasting followed by etching, rinsing and drying and these sub- strates are then individually coated at a coating/baking line. It has thus been necessary to synchronize the etching with the coating/baking because the etched substrates cannot be left for long periods (more than about two days) without detriment to the electrode performance due to air oxidation of the substrate before coating, especially if dust or dirt becomes anchored in the thin oxide film. By precoating the sets of substrates with an improved barrier layer immediately after etching, this bottleneck effect is avoided and the surface-treated substrates can be stored without any risk of further oxidation. Any dust or dirt which may settle on the barrier layer can be easily blown off prior to coating, since it does not get anchored in the film.

Furthermore, the dip-coating procedure of a set of substrates piled against one another is satisfactory for the production of the improved barrier layer oxide film grown up from the substrate. Similar handling is not satisfactory for application of the conventional coatings where an added thickness of each applied coating must be built up over and on top of the film-forming metal base and its very thin surface oxide film.

The electrode base may be a sheet of any film-forming metal, titanium being preferred for cost reasons. Rods, tubes and expanded meshes of titanium or other film-forming metals may likewise be surface treated by the method of the invention. Titanium or other film-forming metal clad on a conducting core can also be used. For most applications, the base will be etched prior to the surface treatment to provide a rough surface giving good anchorage for the subsequently applied electrocatalytic coating. It is also possible to surface-treat porous sintered or plasma-sprayed titanium with the dilute paint solutions in the same manner, but preferably the porous titanium will be only a surface layer on a non-porous base.

The electrodes with an improved barrier layer according to the invention are excellently suited as anodes for chlor-alkali electrolysis. These electrodes have also shown outstanding performance when used for electrowinning in a mixed chloride-sulphate electrolyte giving mixed chlorine and oxygen evolution.

### Best Modes for Carrying Out the Invention

This invention will be further illustrated in the following examples.

### Example I

Coupons measuring 7.5 x 2 cm of titanium available under the trade name "Contimet 30" were degreased, rinsed in water, dried and etched for 1/2 hour in oxalic acid. A paint solution consisting of 6 ml n-propanol, 0.4 ml HCI (concentrated) and 0.1 g of iridium and/or rhodium chloride was then applied by brush to both sides of the coupons in four thin coats. The coupons were dried to evaporate the solvent and then heated in air to 500°C for 10 minutes after each of the first three coats and for 30 mins. after the final coat. This gives a content of about 0.2 to 0.3 g/m² of rhodium and/or iridium (calculated as metal) in the barrier layer depending on the amount of solution in each applied coat, as determined by weight measurement.

A titanium oxide-ruthenium oxide solid solution having a titanium: ruthenium atomic ratio of approximately 2:1 was then applied by brushing on a solution consisting of 6 ml n-propanol, 0.4 ml HCI (concentrated), 3 ml butyl titanate and 1 g RuCI₃ and heating in air at 400°C for 5 mins. (Note: this solution is 10 times more concentrated in terms of precious metal:propanol solvent than is the dilute solution used for producing the barrier layer). This procedure was repeated until the coating was present in thickness of approximately 10 g/m² (i.e. approx. 4 g/m² of Ru metal).

Electrodes so produced as being subjected to comparative electrochemical tests with similar electrodes (a) having a Ti0₂ barrier layer produced by the same procedure but with a paint consisting solely of 6 ml n-propanol and 0.4 ml HCI (concentrated) and (b) having no barrier layer. The initial results indicate that the electrode according to the invention has a greatly superior lifetime in accelerated lifetime tests as anodes in oxygen evolving conditions and, in chlor-alkali electrolysis, should have a lifetime many times-longer than comparative anode (a) and considerably longer than comparative anode (b).

### Example II

A titanium coupon was degreased, rinsed in water, dried, etched and then surface-treated as in Example I with a paint solution containing iridium and ruthenium chlorides in the weight ratio of 2:1 (as metal). The treatment was repeated four times until the titanium dioxide film formed contained an amount of 0.2 g/m² Ir and 0.1 g/m² Ru, both calculated as metal. The heat treatment was carried out at 400°C for 10 minutes after each applied coat. An outer coating of TiO₂ · Ru0₂ was then applied as in Example I. The same comparative electrochemical tests have given the same initial promising results as for Example I.

### Example III

Titanium coupons were degreased, rinsed in water, dried and etched as in Example I and treated with an iridium chloride solution similar to that of Example I. The solution was applied in four thin coats and the coupons were dried to evaporate the solvent and then heated to 480°C for 7 minutes at the end of each coat. The iridium concentration was varied to give a content of 0.3, 0.6 and 0.8 g/m² of iridium (calculated as metal) in the barrier layer.

A titanium dioxide - ruthenium dioxide solution coating was then applied as in Example I, except that the coating thickness corresponded to 20 g/m² (approx. 8 g/m² of Ru metal). These electrodes were subjected to accelerated lifetime tests in oxygen evolving conditions. The maximum lifetimes was observed with the coupon having a barrier layer containing 0.6 g/m² Ir. This represented an increase by a factor of 10.3 of the lifetime of a similar electrode without a barrier layer (or with a barrier layer of Ti0₂ containing no iridium). In comparison, a similar coated electrode with no barrier layer but with the addition of 0.6 g of iridium dispersed in the coating shows only a marginal increase of lifetime.

### Example IV

Electrodes were prepared in a similar manner to Example I, but using a dilute paint containing chlorides of various platinum-group metals, including palladium, platinum and ruthenium alone, as well as rhodium and iridium as previously described, for production of the barrier layer. These electrodes were subjected to comparative lifetime tests as oxygen- evolution anodes. Only the electrodes having a barrier layer containing Rh and/or Ir showed a marked increase in lifetime in this test; combinations of Rh and/or Ir with smaller quantities of the other platinum-group metals or their compounds, in particular Ru and Pd also produced substantial improvements.

### Example V

Titanium coupons were provided with barrier layers containing approx. 0.2 g/m² of iridium and/or rhodium following the procedure of Example I. They were then painted with a solution containing 0.5 g of iridium chloride and 1 g of platinum chloride in 10 ml of isopropyl alcohol and 10 ml of linalool, and heated in an oven to 350°C. An ammonia/hydrogen mixture was then passed for approximately 30 seconds to produce a coating containing 70% Pt and 30% lr. The coating procedure was repeated to build up a coating containing 4 g/m² of the Pt/lr alloy. For similar electrodes coated with less than 7 g/m² of the Pt/lr alloy but without the improved barrier layer, it has been reported that operation at elevated current density produces passivation and at least 7 g/m² must be applied to obtain satisfactory operation over extended periods. This problem is apparently overcome by the electrode according to the invention which operates satisfactorily with a coating of 4 g/m².

### Example VI

Titanium coupons were provided with barrier layers containing approx. 0.2 g/m² of iridium and/or rhodium following the procedure of Example I: A layer of approximately 400 g/m² of titanium oxide was then plasma-sprayed onto the barrier layer, using standard techniques. The plasma-sprayed titanium oxide layer was then coated with coatings containing 2 g/m² (as metal) of ruthenium oxide and/or iridium oxide in various ratios, by painting with a solution of 6 ml propanol and 1 g of RuCI₃ and/or IrCI₃ and heating in air to 500°C for 10 minutes after each coating. Preliminary electrochemical testing indicates that these electrodes should have an extremely long lifetime as anodes in mercury chlor-alkali cells operating at high current densities. From the data published in US Patent 4 140 813, it seems that the electrode of this invention will achieve the same excellent lifetimes with as little as 1/5th of the precious metal loading.

### Example VII

Titanium coupons were provided with barrier layers containing approx. 0.3 g/m² of iridium, rhodium and iridium/ruthenium in a 2:1 weight ratio, following the procedure of Example I (except that in some instances the final heating was prolonged for several hours).

An aqueous solution containing iridium chloride and tantalum chloride (with Ir and Ta metals in an equal weight ratio) was applied by brush over both sides of the coupons in 5, 10 and 15 coats. Each applied coat contained about 0.5 g/m² of iridium. After each coat, the coupons were dried and heated in air for 10 minutes at 450°C, and for 1 hour after the final coat. The resulting coating was a solid solution of iridium and tantalum oxides containing approx. 2.5, 5 and 7.5 g/m² of iridium. The electrodes were tested as anodes in 10% sulfuric acid at 60°C at a current density of 1.2 kA/m², the current being stopped for 15 minutes in each 24-hour period without the electrodes being removed from the acid bath. The initial results indicate a superior performance over similar electrodes on a plain titanium substrate and on a substrate of a titanium-palladium alloy containing 0.15% palladium. The titanium substrate with a barrier layer according to the invention is of course far less expensive than this titanium-palladium alloy and provides a greatly improved resistance to cell shutdown and the passivating action of oxygen evolution. From the preliminary indications, the electrodes according to the invention with a low iridium loading (2.5 g/m² + 0.3 g/m² in the barrier layer) should have an outstanding lifetime compared to similar electrodes without the barrier layer.

## Claims

1. An electrode for use in electrolytic processes comprising a substrate of film-forming metal having a porous electrocatalytic coating comprising at least one platinum-group metal and/or oxide thereof possibly mixed with other metal oxides, in an amount of at least about 2 g/m² of the platinum-group metal(s) per projected surface area of the substrate, and the substrate having below the coating a preformed barrier layer constituted by a surface oxide film grown up from the substrate, characterized in that the preformed barrier layer has rhodium and/or iridium incorporated in the surface oxide film during formation thereof in an amount of up to 1 g/m² (as metal) per projected surface area of the substrate.

2. The electrode of claim 1, wherein the porous electrocatalytic coating consists of a plurality of superimposed layers of micro-cracked configuration.

3. The electrode of claim 2, wherein the porous electrocatalytic coating consists predominantly of a solid-solution of at least one film-forming metal oxide and at least one platinum-group metal oxide.

4. The electrode of claim 3, wherein the porous electrocatalytic coating is a solid solution of ruthenium and titanium oxides having a ruthenium :titanium atomic ratio of from 1:1 to 1:4.

5. The electrode of claim 1, wherein the porous electrocatalytic coating consists predominantly of one or more platinum-group metals.

6. The electrode of claim 5, wherein the porous electrocatalytic coating is a platinum-iridium alloy.

7. The electrode of claim 1, wherein the porous electrocatalytic coating is a plasma-sprayed layer of at least one film-forming metal oxide incorporating the platinum-group metal(s) and/or oxides thereof.

8. The electrode of any preceding claim, wherein the surface oxide film of the barrier layer contains at least one extra added metal in addition to rhodium and/or iridium but in a lesser amount than the rhodium and/or iridium, the total metal content of the barrier layer being up to 1 g/ₘ2_{.}

9. The electrode of claim 8, wherein said film contains up to 0.5 g/m² of iridium and ruthenium in a weight ratio of about 2:1.

10. The electrode of any preceding claim, wherein the substrate is of titanium and the surface oxide film is predominantly rutile titanium dioxide.

11. A method of manufacturing an electrode for use in electrolytic processes, comprising forming a barrier layer on a substrate of film-forming metal and applying over the barrier layer a porous outer electro-catalytic coating comprising at least one platinum-group metal and/or oxide thereof possibly mixed with other oxides, in an amount of at least about 2 g/m² of the platinum-group metal(s) per projected surface area of the substrate, characterized in that the barrier layer is formed by applying to the substrate one or more coats of a very dilute (as hereinafter defined) acid solution containing a thermodecomposable compound of rhodium and/or iridium, drying and heating the or each coat to form on the substrate a surface film of film-forming metal oxide and simultaneously at least partially decompose said compounds, the or each applied coat of said very dilute solution containing a quantity of said compound that is substantially fully absorbed in the surface film formed during heating, and the number of applied coats being such that the barrier layer so formed contains up to 1.0 g/m² of rhodium and/or iridium per projected surface area of the substrate.

12. The method of claim 11, wherein the or each applied coat of the solution contains up to 0.2 g/m² of rhodium and/or iridium metal per projected surface area of the substrate.

13. A method of manufacturing an electrode for use in electrolytic processes, comprising forming a barrier layer on a substrate of film-forming metal and applying over the barrier layer a porous outer electrocatalytic coating comprising at least one platinum group metal and/or oxide thereof possibly mixed with other oxides, in an amount of at least about 2 g/m² of the platinum group metal(s) per projected surface area of the substrate, characterized in that the barrier layer is formed by applying to the substrate several coats each containing up to 0.2 g/m² (as metal per projected surface area of the substrate) of a thermodecomposable compound of rhodium and/or iridium in a solution which attacks the film-forming metal substrate, and heating after drying each coat to produce a barrier layer of oxide of the film-forming metal containing up to 1.0 g/m² of iridium and/or rhodium.

14. The method of any one of claims 11 to 13, wherein from 2 to 5 coats of the dilute solution are applied each followed by heating to between about 300° and 600°C for about 5 to 15 minutes, the final coat possibly being heated for a longer period.

15. The method of any one of claims 11 to 14, wherein the heating is carried out to incompletely decompose said compound.

16. The method of any one of claims 11 to 15, wherein the porous outer electrocatalytic coating is formed by applying over the preformed barrier layer a plurality of coats of a relatively concentrated solution containing a thermodecomposable platinum group metal compound and heating.

17. The method of claim 16, wherein each applied outer coat contains at least 0.4 g/m² of platinum group metal per projected area of the substrate base.

18. The method of any one of claims 11 to 15, wherein the porous outer electrocatalytic coating is applied by plasma-spraying.

19. The method of any one of claims 11 to 15, wherein the porous outer electrocatalytic coating is applied by plasma spraying at least one film-forming metal oxide over the preformed barrier layer and subsequently incorporating the platinum group metal(s) and/or oxides thereof in the plasma-sprayed film-forming metal oxide.

20. The method of any one of claims 11 to 19, wherein a set of electrode substrates are subjected together to a series of pretreatments including etching and formation of the barrier layer by dip-coating the set of substrates in said dilute solution and heating the set of sub- strates, and thereafter the outer electro- catalytic coating is applied to the substrates one at a time.

21. The electrode produced by the method of any one of claims 11 to 20.

22. Use of the electrode of any one of claims 1 to 10 or 21 as anode in chlor-alkali electrolysis.

## Patentansprüche

1. Elektrode zum Gebrauch in einem elektrolytischen Prozess mit einem Substrat aus einem filmformenden Metall und mit einer porösen elektrokatalytischen Schicht aus mindestens einem Platingruppenmetall und/oder einem Oxid hiervon welches möglicherweise mit anderen Metalloxiden gemischt ist, wobei die Menge des Platingruppenmetalls mindestens 2g/m² der projektierten Oberfläche des Substrats beträgt, und wobei das Substrat unter dieser Schicht eine vorgeformte Schutzschicht aus einem Oberflächenoxidfilm aufweist welcher auf dem Substrat gewachsen ist, dadurch gekennzeichnet dass die vorgeformte Schutzschicht Rhodium und/oder Iridium aufweist, welche in den Oberflächenoxidfilm während seiner Entstehung in einer Menge von bis zu einem Gramm (als Metall) pro _{M}² der projektierten Oberfläche des Substrats eingebettet wurden.

2. Elektrode nach Anspruch 1 wobei die poröse elektrokatalytische Schicht aus einer Mehrzahl von übereinanderliegenden Schichten mikroskopisch rissiger Struktur besteht.

3. Elektrode nach Anspruch 2 wobei die poröse elektrokatalytische Schicht hauptsächlich aus einer festen Lösung zumindest eines filmformenden Metalloxids und mindestens eines Platingruppenmetalloxids besteht.

4. Elektrode nach Anspruch 3 worin die poröse elektrokatalytische Schicht eine feste Lösung von Ruthenium und Titanoxid besteht, welche ein Atomverhältnis von Ruthenium zu Titan von 1:1 bis 1:4 aufweisen.

5. Elektrode nach Anspruch 1 worin die poröse elektrokatalytische Schicht hauptsächlich aus einem oder mehreren Platingruppenmetallen besteht.

6. Elektrode nach Anspruch 5 worin die poröse elektrokatalytische Schicht eine Platin-Iridium-Legierung ist.

7. Elektrode nach Anspruch 1 worin die poröse elektrokatalytische Schicht aus einer plasmagespritzten Schicht aus mindestens einem filmformenden Metalloxid besteht, welche Platingruppenmetalle und/oder Oxide hiervon aufweist.

8. Elektrode nach einem der vorhergehenden Ansprüche worin der Oberflächenoxidfilm der Schutzschicht zusätzlich zu Rhodium und/oder Iridium ein weiteres Metall aufweist, welches in einer geringeren Menge als des Rhodium und/oder das Iridium vorliegt, wobei der gesamte Metallinhalt der Schutzschicht bis zu einer Gramm pro m² beträgt.

9. Elektrode nach Anspruch 8 worin der Film bis zu 0.5 Gramm pro m² Iridium und Ruthenium in einem Gewichtsverhältnis von etwa 2:1 aufweist.

10. Elektrode nach einem der vorhergehenden Ansprüche worin das Substrat aus Titan besteht und der Oberflächenfilm vorwiegend aus rutilem Titandioxid besteht.

11. Verfahren zur Herstellung einer Elektrode zum Gebrauch in elektrolytischen Prozessen wobei eine Schutzschicht auf einem Substrat aus einem filmformenden Metall und über der Schutzschicht eine poröse äussere elektrotatalytische Schicht aus mindesten einem Platingruppenmetall und/oder Oxiden hiervon, welche möglicherweise mit anderen Oxiden vermischt sind, gebildet wird, wobei das Substrat mindestens etwa 2 Gramm des Platingruppenmetalls pro m² der projektierten Oberfläche des Substrats enthält, dadurch gekennzeichnet dass die Schutzschicht durch Aufbringen von einer oder mehreren Schichten eines stark verdünnten (wie weiter unten definiert) Säurelösung aufgebracht wird, welche eine thermisch zersetzbare Verbindung von Rhodium und/ oder Iridium aufweist, Trocknen und Aufheizen der Schicht(en) um auf dem Substrat einen Oberflächenfilm des filmformenden Metalloxids zu formen, und gleichzeitig die genannte Verbindung zumindest teilweise zu zersetzen, wobei die bzw. jede der aufgebrachten Schichten dieser stark verdünnten Lösung eine Menge der genannten Verbindung enthält, welche im wesentlichen vollständig im Oberflächenfilm während des Heizens absorbiert wird, wobei die Anzahl der aufgebrachten Schichten derart ist, dass die derart geformte Schutzschicht bis zu einem Gramm Rhodium und/oder Iridium pro m² der projektierten Oberfläche des Substrats enthält.

12. Verfahren nach Anspruch 11 worin die oder jede aufgebrachte Schicht der Lösung bis zu 0.2 g Rhodium oder Iridium Metall pro m² der projektierten Oberfläche des Substrats enthält.

13. Verfahren zur Herstellung einer Elektrode für den Gebrauch in elektrolytischen Prozessen wobei eine Schutzschicht auf einem Substrat eines filmformenden Metalls und über dieser Schutzschicht eine poröse äussere elektrokatalytische Schicht aufgebracht wird, welche zumindest ein Platingruppenmetall und/oder Oxide hiervon aufweist, welche möglicherweise mit anderen Oxiden gemischt sind, wobei das Substrat mindestens etwa 2g Platingruppenmetall(e) pro m² der projektierten Oberfläche aufweist, dadurch gekennzeichnet dass die Schutzschicht durch Aufbringen verschiedener Schichten auf des Substrat hergestellt ist, von denen jede bis zu 0.2g (als Metall pro m² der projektierten Oberfläche des Substrats) einer thermisch zersetzbaren Verbindung von Rhodium und/oder Iridium in einer Lösung aufweist, welche das filmformende Metallsubstrat angreift, und aufheizen jeder Schicht nach Trocknung un eine Schutzschicht eines Oxids des filmformenden Materials zu erzeugen, welche bis zu 1 g Iridium und/oder Rhodium pro m² aufweist.

14. Verfahren nach einem der Ansprüche 11 1 bis 13 wobei zwischen 2 und 5 Schichten der verdünnten Lösung aufgebracht werden, wovon jede hernach auf zwischen 300 und 600°C während 5 bis 15 Minuten aufgeheizt wird, wobei die letzte Schicht möglicherweise für eine längere Zeitspanne aufgeheizt wird.

15. Verfahren nach einem der Ansprüche 11 1 bis 14 wobei das Heizen derart ausgeführt wird, dass die genannte Verbindung unvollständig zersetzt wird.

16. Verfahren nach einem der Ansprüche 11 1 bis 15 worin die poröse äussere elektrokatalytische Schicht durch Aufbringen einer Mehrzahl von Schichten einer relativ konzentrierten Lösung mit einer themisch zersetzbaren Platingruppenmetallverbindung auf das Substrat und Aufheizen hergestellt wird.

17. Verfahren nach Anspruch 16 wobei jede aufgebrachte äussere Schicht mindestens 0.4g des Platingruppenmetalls pro m² der projektierten Oberfläche der Substratunterlage enthält.

18. Verfahren nach einem der Ansprüche 11 1 bis 15 wobei die poröse äussere elektrokatalytische Schicht durch Plasmaspritzen aufgebracht wird.

19. Verfahren nach einem der Ansprüche 11 bis 15 worin die poröse äussere elektrokatalytische Schicht durch Plasmaspritzen mindestens eines filmformenden Metalloxids auf die vorgeforme Schutzschicht und nachfolgendes Einbringen des Platingruppenmetalls und/oder Oxiden hiervon in das plasmagespritzte filmformende Metalloxid hergestellt wird.

20. Verfahren nach einem der Ansprüche 11 1 bis 19 wobei ein Satz von Elektrodensubstraten zusammen einer Reihe von Vorbehandlungen unterzogen wird, welche Ätzen und die Formation einer Schutzschicht durch Eintauchen des Satzes von Substraten in die genannte verdünnte Lösung und Aufheizen des Satzes von Substraten umfassen, wobei die äusseren elektrokatalytischen Schicht einzeln auf jedes Substrat aufgebracht werden.

21. Elektrode dadurch gekennzeichnet, dass sie durch das Verfahren nach einem der Ansprüche 11 bis 20 hergestellt ist.

22. Gebrauch einer Elektrode nach einem der Ansprüche 1 bis 10 oder 21 als Anode für die Chlor-Alkali Elektrolyse.

## Revendications

1. Electrode à utiliser dans des procédés électrolytiques comprenant un support en métal apte à former une pellicule qui présente une surface extérieure électrocatalytique active ayant la forme d'une pellicule superficielle faisant corps avec le support en métal apte à former une pellicule et contenant un métal du groupe du platine ou un composé d'un tel métal en tant qu'électrocatalyseur, caractérisée en ce qu'on forme la surface extérieure électrocatalytique en appliquant à la surface du support en métal apte à former une pellicule au moins une couche d'une solution d'au moins un composé thermodécomposable d'un métal un groupe du platine, on sèche et on chauffe chaque couche appliquée pour décomposer le ou les composés d'une manière semblable à des procédés connus pour la formation de revêtements de métaux du groupe du platine et d'oxydes de ces métaux, la solution contenant un agent qui attaque le support en métal apte à former une pellicule et qui convertit du métal du support en ions qui sont convertis en un composé du métal apte à former une pellicule pendant la phase de chauffage, la concentration du dit agent et du ou des composés du métal du groupe du platine dans la solution et le nombre de couches appliquées étant tels que, pendant le chauffage de chaque couche, y compris celui de la dernière, l'électrocatalyseur formé à partir du composé décomposé est incorporé complètement à la pellicule superficielle de composé en métal apte à former une pellicule formée à partir du support.

2. Electrode suivant la revendication 1, caractérisée en ce que le pellicule superficielle du support en métal apte à former une pellicule est en oxyde.

3. Electrode suivant la revendication 1, caractérisée en ce que la pellicule superficielle du support en métal apte à former une pellicule est en carbure, en nitrure, en hydrure ou en borure.

4. Electrode suivant la revendication 1, 2 ou 3, caractérisée en ce que le support de l'électrode a la forme d'une feuille et la pellicule superficielle contient jusqu'à 0,5 g de l'électrocatalyseur, exprimé en métal, par mètre carré de surface projetée du support d'électrode.

5. Elektrode suivant la revendication 1, 2 ou 3, caractérisée en ce que la pellicule contient de l'iridium et/ou du rhodium sous la forme de métal ou d'oxyde..

6. Elektrode suivant la revendication 1, 2 ou 3, caractérisée en ce que la pellicule contient (a) de l'iridium et/ou du rhodium, et (b) du ruthénium sous la forme de métaux ou d'oxydes en un rapport en poids des métaux (a):(b) de 4:1 à 1:4.

7. Elektrode suivant la revendication 1, 2, 3, 5 ou 6, caractérisée en ce que le support d'électrode est fait de particules.

8. Electrode à utiliser dans des procédés électrolytiques, caractérisée en ce qu'elle comprend des particules d'un métal apte à former une pellicule comportant chacune une pellicule superficielle électrocatalytique et électroconductrice d'oxyde du métal apte à former une pellicule faisant partie intégrante de la particule et contenant un électrocatalyseur en métal du groupe du platine.

9. Electrode suivant la revendication 7 ou 8, caractérisée en ce que les particules sont supportées sur un support conducteur.

10. Electrode suivant la revendication 7 ou 8, caractérisée en ce que les particules sont associées à un élément d'alimentation de courant.

11. Procédé pour former une électrode à utiliser dans des procédés électrolytiques comprenant un support en métal apte à former une pellicule présentant une surface extérieure électrocatalytique active ayant la forme d'une pellicule superficielle faisant corps avec le support en métal apte à former une pellicule et contenant un métal du groupe du platine ou un composé d'un tel métal à titre d'électro-, catalyseur, caractérisé un ce qu'on applique à la surface du support en métal apte à former la pellicule au moins une couche d'une solution d'au moins un composé thermodécomposable d'un métal du groupe du platine, on sèche et on chauffe chaque couche appliquée pour décomposer le ou les composés d'une manière semblable à des procédés connus pour la formation de revêtements de métaux du groupe du platine et d'oxydes et ces métaux, la solution contenant un agent qui attaque le support en métal apte à former une pellicule et qui convertit du métal du support en ions qui sont convertis en un composé du métal apte à former une pellicule pendant la phase de chauffage, la concentration du dit agent et du ou des composés de métal du groupe du platine dans la solution et le nombre de couches appliquées étant tels que, pendant le chauffage, de chaque couche, y compris de la dernière, l'électrocatalyseur formé à partir du composé décomposé est incorporé entièrement à la pellicule superficielle de composé en métal apte à former une pellicule formée à partir du support.

12. Procédé suivant la revendication 11, caractérisé en ce que le support d'électrode a la forme d'une feuille et chaque couche appliquée de la solution contient jusqu'à 0,2 g, exprimé en métal de composé d'iridium, de rhodium et/ou de ruthénium par mètre carré de surface projetée du support d'électrode.

13. Procédé suivant la revendication 11 ou 12, caractérisé en ce que la solution contient des composés de (a) iridium et/ou rhodium, et (b) ruthénium en un rapport en poids des métaux (a) : (b) de 4: 1 1:4.

14. Procédé suivant la revendication 12, caractérisé en ce qu'on applique deux à cinq couches de la solution, chaque application étant suivie d'un chauffage à une température comprise entre environ 400 et 600°C pendant environ 5 à 15 minutes, la couche finale étant éventuellement chauffée pendant une pédiode plus longue.

15. Procédé suivant la revendication 14, caractérisé en ce que la pellicule superficielle finale contient jusqu'à 0,5 g de l'électrocatalyseur, exprimé en métal, par mètre carré de surface projetée du support d'électrode.

16. Procédé suivant la revendication 11, caractérisé en ce que la solution contient le dit agent et la composé de métal du groupe du platine en un rapport molaire de 1:1 à 100:1.

17. Procédé suivant la revendication 16, caractérisé en ce que le rapport molaire est choisi entre 3:1 et 30:1.

18. Procédé suivant l'une quelconque des revendications 11, 13, 16 et 17, caractérisé en ce que le support d'électrode est particulaire.

19. Procédé suivant la revendication 18, caractérisé en ce que la phase de séchage est effectuée en au moins deux stades séparés pour éliminer tout solvant du métal particulaire apte à former une pellicule.

20. Procédé suivant la revendication 18 ou 19, caractérisé en ce qu'il comprend une étape supplémentaire qui consiste à appliquer sur un support conducteur le métal particulaire apte à former une pellicule active en surface.

21. Procédé suivant l'une quelconque des revendications 11 à 20, caractérisé en ce qu'on effectue le chauffage à l'air pour former une pellicule superficielle d'oxyde du métal apte à former une pellicule.

22. Procédé suivant l'une quelconque des revendications 11 à 20, caractérisé en ce que le chauffage est effectué dans une atmosphère non oxydante contenant du carbone, de l'azote, de l'hydrogène ou du bore pour former une pellicule superficielle de carbure, nitrure, hydrure ou borure de métal apte à former une pellicule.
